

1

2,966,390

**PROCESS FOR THE PRODUCTION OF ETCHED TEXTILE MATERIAL CONTAINING SYNTHETIC CELLULOSE FIBERS**

Franz Hoelkeskamp, Wuppertal-Langerfeld, and Heinz Hipp, Wuppertal-Barmen, Germany, assignors to J. P. Bemberg Aktiengesellschaft, Wuppertal-Oberbarmen, Germany

No Drawing. Filed Aug. 6, 1956, Ser. No. 602,446

Claims priority, application Germany Aug. 8, 1955

11 Claims. (Cl. 18—54)

This invention relates to a process for the production of an etched textile material containing synthetic cellulose fibers, and more particularly to a process for the preparation and production of a textile material containing dyed synthetic cellulose fibers in which the dyestuff pigment is partially reduced or decomposed.

It is a familiar practice to apply suitable dyestuffs to finished textiles in the form of threads, yarns, cloth, fabric or the like containing synthetic cellulose fibers, and then etching the textile material in a subsequent manufacturing operation. The etching step of the process includes the decomposition of dyestuff pigment by reaction with a reducing agent in order to partially remove or destroy the dye at various locations or places on the textile material. It is also a familiar practice to apply insoluble dyestuff pigments to a spinning solution shortly before spinning synthetic filaments or fibers therefrom in order to produce an internally dyed fiber which can be made into ultra-fast dyed textile materials.

The principal object of the present invention is to provide a process for the production of an etched and at the same time an ultra-fast dyed textile material containing synthetic cellulose fibers. Other objects and advantages of the invention will become more apparent upon a consideration of the following description of the invention.

In accordance with the invention, this principal object is achieved by dispersing a very finely divided, water-insoluble dyestuff pigment in a cellulosic spinning solution, the dyestuff pigment being capable of being decomposed by a reducing agent, spinning internally dyed synthetic cellulose fibers from the spinning solution, and etching a textile material containing the internally dyed fibers by reaction with a reducing agent.

A very fine distribution or dispersion of the dyestuff pigments in the cellulosic spinning solution is advantageously obtained by employing dyestuff pigments having a particle size of not more than five microns. Correspondingly, internally dyed fibers or filaments are obtained in which the embedded dyestuff pigments, even in the interior of the fibers, can be etched by reaction with a reducing agent. A finely dispersed and highly uniform suspension of the dyestuff pigments in the spinning solution is further obtained by the use of a suitable emulsifying agent. Such emulsifiers are well known in the art, and only a small quantity is required to give a satisfactory dispersion of the water-insoluble pigment.

Naturally, the dyestuff pigment selected for the process of the invention should be resistant or inert to the prevailing operating conditions ordinarily employed in spinning synthetic cellulose fibers. Thus, a dyestuff pigment to be dispersed in a viscous spinning solution should be both alkali and acid resistant and should also be fast to sulfur compounds. Where conventional chemical treatments of the fibers and/or textile material, such as soaping, desulfurizing and the like are employed, the dyestuff pigment is, of course, preferably selected so

2

as to remain fast to such treatment. These modifications and limitations of the dyestuff employed will be readily apparent to those skilled in the art and are mentioned herein merely as an aid in selecting suitable dyestuffs without departing from the spirit and scope of the invention.

Examples of particular dyestuffs which are especially useful in the process of the invention include water-insoluble, etchable dyestuff pigments obtained as the reaction products or coupling products of naphthols with diazotized aromatic amines, these reaction products being commonly classed as azoic dyestuffs. The group of Celliton dyestuffs which are water-insoluble and also etchable or decomposable by reduction are likewise suitable for employment in the present process (e.g., see Dyestuff Tables of Schultz, 7th printing, volume 2, pages 44—45; supplemental volume 1, pages 75 and 76; and supplemental volume 2, pages 138—143).

Among the azoic dyestuffs which can be utilized as dyestuff pigments, those which have been found to be particularly advantageous include the following combinations of a diazotized aromatic amine component with a naphthol component:

25 Fast Black Salt G, m-nitranilide of 2,3-oxynaphthoic acid;  
Fast Gold Orange Salt GR, o-toluidide of 2,3-oxynaphthoic acid:

Pigment Fast (Schultz No. 85)



35 Oil Red (Schultz No. 118)



40 45 Oil Vermillion (Schultz No. 149)



50 55 Polarorange R conc. (Schultz No. 367)



60 65 Celliton dyestuff pigments which have been found to be particularly useful in the practice of the invention include all those Celliton dyestuff pigments which are insoluble in water and etchable with a reducing agent. They may be selected from the group of Celliton dyestuffs classified in Dyestuff Tables of Schultz, 7th printing, volume 2, pages 1—233.

The dyestuff pigments are preferably first prepared as aqueous suspension and this suspension then added to the spinning solution. In order to ensure a uniform distribution of the dyestuff pigments as a suspension in an aqueous solution, the naphthol and diazotized amine of an azoid dyestuff should be linked or combined in an aqueous media in the presence of an emulsification agent. Likewise, in preparing an aqueous suspension of a Celliton dyestuff, the dyestuff is preferably first dissolved in alcohol after which the alcoholic solution is mixed with water containing a suitable emulsification agent. The alcohol can be vaporized so that the dyestuff pigment remains as a fine suspension in the aqueous media. The emulsification agents employed are well known in the art and include, for example, ethoxylated fatty alcohols or ethoxylated alcoyphenols.

A sufficient quantity of the dyestuff contained in an aqueous suspension is added to the cellulosic spinning solution to give the desired degree of coloring to the finished textile material. Generally, it is preferred that the concentration of dyestuff pigments amount to from about 1% to 5%, especially about 2% to 4%, by weight of the cellulose content of the spinning solution.

The spinning solution containing the dispersed dyestuff is extruded in a conventional manner into continuous filaments which can then be made into a textile material, as by collecting a plurality of fibers in the form of a thread or yarn and weaving the fibers into a fabric, cloth, or the like. Internally dyed fibers or filaments are thus contained in an etchable textile material, i.e., a textile material containing synthetic cellulose fibers in which there has been internally incorporated a dyestuff pigment capable of being partially reduced or decomposed.

The etching step of the process is carried out by subjecting the textile material to the action of a reducing agent, preferably a strong reducing agent such as sodium hydrosulfite. Other suitable reducing agents include hydrazines and formaldehyde sodiumsulfoxylate, known as "Rongalite."

The invention is further illustrated by the following examples in which the description includes (a) the production of an aqueous suspension containing the finely dispersed dyestuff pigment, and (b) the preparation of the spinning solution. It is to be understood that the examples are illustrative only and are not intended to limit the scope of the invention. Parts are parts by weight unless otherwise specified.

#### Example 1

(a) 33.9 parts of a diazotized amine (Fast Black Salt G, see Dyestuff Tables of Schultz, 7th printing, supplementary volume 1, page 94) are dissolved in 1000 parts of hot water with the addition of 89 parts of acetic acid and 1.4 parts of an emulsifying agent as an ethoxylated oleyl alcohol with 10-20 moles ethyleneoxide. With very strong stirring there is added a solution of 19 parts of m-nitranilide of 2,3-oxynaphthoic acid and an equivalent quantity of caustic soda solution in 2000 parts of water. An aqueous suspension of a water-insoluble dyestuff pigment is thus formed having a pH of 8.2.

(b) 3,120 parts of this suspension, which contains 52.9 parts of the dyestuff pigment, are added with constant stirring to 14,650 parts of a cuprammonium solution having a cellulose content of 12% by weight. After the solution has been well homogenized, 1,730 parts of water are further added to give a cellulose content of 9% by weight of the spinning solution. The spinning solution, which contains 3% of dyestuff pigments with reference to the cellulose content, is then spun by extrusion in the usual manner to form a plurality of internally dyed continuous filaments.

The internally dyed filaments are woven into a fabric, and the fabric is then etched by means of sodium hydrosulfite. Various portions of the fabric are etched where the sodium hydrosulfite has decomposed the dyestuff pig-

ment. The fabric is also ultra-fast dyed, having a permanent, solid coloring.

#### Example 2

(a) 50.3 parts of a diazotized amine (Fast Gold Orange Salt GR, see Dyestuff Tables of Schultz, 7th printing, supplementary volume 2, page 178) are dissolved in 1000 parts of hot water with the addition of 16.2 parts of acetic acid and 1.5 parts by weight of a suitable emulsifier as iso-dodecylphenol with 6 moles ethyleneoxide. To this there is added together with intensive stirring a solution consisting of 16.3 parts of the o-toluidide of 2,3-oxynaphthoic acid in 2000 parts of water and an equivalent amount of caustic soda solution. The pH is set at 8.2 to 8.3 in the resulting suspension.

(b) 1,500 parts of the dyestuff suspension thus prepared, which contains 33.3 parts of the dyestuff pigment, are added with constant stirring to 9,250 parts of a viscose spinning solution which contains 9% by weight of cellulose. After the dyestuff pigments are evenly distributed, 3,150 parts of water are further added so that a solution ready for spinning is provided having a content of 6% by weight of cellulose. The concentration of the dyestuff pigment amounts to 4% by weight with reference to the cellulose.

From the internally dyed spun filaments, a textile fabric is produced which can be etched by means of sodium hydrosulfite.

#### Example 3

(a) 10 parts of Celliton Fast Yellow G (see Dyestuff Tables of Schultz, 7th printing, volume 2, page 45) are dissolved in 85 parts of 96% alcohol as the solution is warmed. The initial dye solution is introduced drop by drop into 1000 parts of water being vigorously stirred, the water containing 0.1% of an emulsifier, as in Example 2, Lavagent. A finely dispersed dyestuff suspension results. The alcohol is vaporized and the suspension is set at a pH value of 8.2.

(b) 3,120 parts of this suspension are added to 14,650 parts of a cuprammonium spinning solution which has a cellulose content of 12% by weight. The remainder of the process is carried out in accordance with the procedure described in Example 1(b) to obtain a fabric etched by sodium hydrosulfite.

#### Example 4

(a) An aqueous suspension of a water-insoluble dyestuff pigment is produced in the same manner as Example 1.

(b) This suspension is added to a viscose spinning solution with 6.8% cellulose and 6.5% sodium hydroxide in such a quantity that the spinning solution will contain 3% of dyestuff pigment with reference to the cellulose content. The spinning process is accomplished in the usual manner.

The internally dyed filaments are woven into a fabric, which is then etched by means of sodium hydrosulfite.

#### Example 5

(a) An aqueous suspension of a water-insoluble dyestuff pigment is produced in the same manner as Example 2 except that the following dyestuff pigments were employed:

Oil Vermillon (Schultz No. 149)  
Pigment Fast (Schultz No. 85)  
Polarorange R conc. (Schultz No. 367)

(b) When the textile material is being etched by means of sodium hydrosulfite the blue-red color of Oil Vermillon (Schultz No. 149) turns to a scarlet shade.

The process of the invention gives the possibility to produce an etched and at the same time ultra-fast dyed textile material. A further advantage of the invention is that it enables the production of a colored textile material with etched designs of clear contours, which remain unchanged even when washed several times. If the

etching process will be accomplished in several steps one gets different color shades also with clear contours.

The invention is hereby claimed as follows:

1. A process for the production of an etched textile material containing synthetic cellulose fibers which comprises dispersing a very finely divided, water-insoluble organic dyestuff in a cellulosic spinning solution, said dyestuff being capable of being decomposed by a reducing agent, spinning internally dyed synthetic cellulose fibers from said spinning solution, and etching a textile material containing said internally dyed fibers by reaction with a reducing agent.

2. A process as defined in claim 1 wherein the dyestuff is an azoic dyestuff.

3. A process as defined in claim 1 wherein the dyestuff has a particle size of not more than five microns.

4. A process as defined in claim 1 wherein the dispersion of the dyestuff is accomplished in the presence of an emulsifying agent.

5. A process for the production of an etched textile material containing synthetic cellulose fibers which comprises dispersing a very finely divided, water-insoluble organic dyestuff in the presence of an emulsifying agent in a cellulosic spinning solution such that the quantity of said dyestuff is from about 1% to 5% by weight of the cellulose content of said spinning solution, said dyestuff being capable of being decomposed by a reducing agent, spinning internally dyed synthetic cellulose fibers from said spinning solution, and etching a textile material containing said internally dyed fibers by reaction with a reducing agent.

6. A process for the production of an etched textile material containing synthetic cellulose fibers which comprises dispersing a very finely divided, water-insoluble organic dyestuff in the presence of an emulsifying agent in a cellulosic spinning solution such that the quantity of said dyestuff is from about 2% to 4% by weight of the

cellulose content of said spinning solution, said dyestuff being capable of being decomposed by a reducing agent, spinning internally dyed synthetic cellulose fibers from said spinning solution, and etching a textile material containing said internally dyed fibers by reaction with a strong reducing agent.

7. A process as defined in claim 6 wherein the reducing agent is sodium hydrosulfite.

8. A process as defined in claim 6 wherein the reducing agent is hydrazine.

9. A process as defined in claim 6 wherein the reducing agent is formaldehyde sodiumsulfoxylate.

10. A process of producing color-fast etched designs on a textile material containing synthetic cellulose fibers which comprises applying a reducing agent to selected portions of said textile material in which the cellulose fibers have been uniformly colored by dispersing a finely divided, water-insoluble organic dyestuff in an aqueous cellulosic spinning solution prior to spinning said fibers, said dyestuff being capable of being decomposed by said reducing agent.

11. A process as defined in claim 10 wherein the dyestuff is an azoic dyestuff.

25

#### References Cited in the file of this patent

#### UNITED STATES PATENTS

|           |                |               |
|-----------|----------------|---------------|
| 2,143,883 | Kline et al.   | Jan. 17, 1939 |
| 2,166,741 | Karplus        | July 18, 1939 |
| 2,210,774 | Perrin et al.  | Aug. 6, 1940  |
| 2,261,295 | Schlack        | Nov. 4, 1941  |
| 2,345,345 | Koch           | Mar. 28, 1944 |
| 2,385,885 | Seymour et al. | Oct. 2, 1945  |
| 2,457,808 | Dort           | Jan. 4, 1949  |
| 2,583,192 | Waite          | Jan. 22, 1952 |
| 2,650,168 | Van Dijk       | Aug. 25, 1953 |